# EUROPEAN PATENT SPECIFICATION

(11) **EP 3 109 330 B1**
(45) Date of publication and mention of the grant of the patent: **22.08.2018**
(21) Application number: 15751393.8
(22) Date of filing: 03.02.2015
(51) Int. Cl.: C21D 9/46, C21D 1/76, C22C 38/00, C22C 38/06, C22C 38/58

(54) **METHOD FOR PRODUCING HIGH-STRENGTH STEEL PLATE**
VERFAHREN ZUR HERSTELLUNG VON HOCHFESTEM STAHLBLECH
PROCÉDÉ DE PRODUCTION DE TÔLE D'ACIER À HAUTE RÉSISTANCE

(30) Priority: 18.02.2014 JP 2014028030
(43) Date of publication of application: 28.12.2016
(73) Proprietor: JFE Steel Corporation, Tokyo 100-0011 (JP)
(72) Inventor: FUSHIWAKI, Yusuke, Tokyo 100-0011 (JP); KAWASAKI, Yoshiyasu, Tokyo 100-0011 (JP)
(74) Representative: Stebbing, Timothy Charles
(86) International application number: PCT/JP2015/000460
(87) International publication number: WO 2015/125422

(56) References cited:
- EP-A1- 2 623 631
- WO-A1-2013/140729
- WO-A1-2014/017010
- JP-A- 2006 183 131
- JP-A- 2007 262 463
- JP-A- 2010 255 110
- JP-A- 2012 251 239
- JP-A- 2013 124 382
- JP-A- 2013 194 271
- JP-A- 2014 015 675

## Description

### Technical Field

The present invention relates to a high-strength steel sheet that has excellent chemical conversion treatability and corrosion resistance after electrodeposition coating even when the content of Si or Mn is high. The present invention also relates to a method for manufacturing the high-strength steel sheet.

### Background Art

In recent years, from the viewpoint of improving the fuel efficiency of automobiles and the viewpoint of enhancing the crash safety of automobiles, there have been growing demands that automobile bodies are lightened and strengthened in such a manner that automobile body materials are strengthened and are thereby gauged down. Therefore, the application of high-strength steel sheets to automobiles is promoted.

In usual, steel sheets for automobiles are used after being coated. The steel sheets are subjected to a chemical conversion treatment, called a phosphate treatment, as a pretreatment for coating. The chemical conversion treatment of a steel sheet is one of important treatments for ensuring corrosion resistance after coating.

The addition of Si and Mn is effective in increasing the strength and ductility of a steel sheet. However, even in the case where the steel sheet is annealed in a reducing N₂ + H₂ gas atmosphere in which Fe is not oxidized (Fe oxides are reduced), Si and Mn are oxidized during continuous annealing to form surface oxides (such as SiO₂ and MnO, hereinafter referred to as selective surface oxides) selectively containing Si or Mn in the outermost surface layer of the steel sheet. Since the selective surface oxides inhibit the formation reaction of a chemical conversion coating during a chemical conversion treatment, a fine region (hereinafter referred to as a lack of hiding in some cases) where no chemical conversion coating is produced is formed, leading to a reduction in chemical conversion treatability.

Patent Literature 1 discloses a method for forming a 20-1,500 mg/m² iron coating layer on a steel sheet by an electroplating process as a conventional technique for improving the chemical conversion treatability of a steel sheet containing Si and Mn. However, this method has a problem that an electroplating line is necessary and therefore the increase in number of steps causes an increase in cost.

Phosphate treatability is enhanced by regulating the Mn/Si ratio as described in Patent Literature 2 or by adding Ni as described in Patent Literature 3. However, the effect depends on the content of Si or Mn in a steel sheet; hence, further improvements are probably necessary for steel sheets with a high Si or Mn content.

Patent Literature 4 discloses a method in which an internal oxidation layer made of an Si-containing oxide is formed within a depth of 1 µm from the surface of an underlayer of a steel sheet by controlling the dew point at -25°C to 0°C during annealing such that the proportion of the Si-containing oxide in a length of 10 µm in a surface of the steel sheet is 80% or less. However, in the method disclosed in Patent Literature 4, the control of the dew point is difficult and stable operation is also difficult because an area where the dew point is controlled is based on the whole inside of a furnace. In the case where annealing is performed by the unstable control of the dew point, the distribution of internal oxides formed in a steel sheet is uneven and unevenness in chemical conversion treatability (a lack of hiding in the whole or a portion) may possibly be caused in a longitudinal or transverse direction of the steel sheet. Alternatively, in the case of enhanced chemical conversion treatability, there is a problem in that corrosion resistance after electrodeposition coating is poor because the Si-containing oxide is present directly under a chemical conversion coating.

Patent Literature 5 discloses a method in which an oxide film is formed on a surface of a steel sheet in an oxidizing atmosphere by increasing the temperature of the steel sheet to 350°C to 650°C and the steel sheet is heated to a recrystallization temperature in a reducing atmosphere and is then cooled. However, in this method, the thickness of the oxide film formed on the steel sheet surface is uneven depending on an oxidation process, oxidation does not occur sufficiently, or the oxide film is too thick so that the oxide film remains or peels off during the subsequent annealing in the reducing atmosphere and therefore surface properties are poor in some cases. In an example, a technique for performing oxidation in air is described. However, oxidation in air has a problem that, for example, thick oxides are produced and subsequent reduction is difficult or a reducing atmosphere with a high hydrogen concentration is necessary.

Patent Literature 6 discloses a method in which an oxide film is formed on a surface of a cold-rolled steel sheet containing 0.1% or more Si and/or 1.0% or more Mn on a mass basis at a steel sheet temperature of 400°C or higher in an atmosphere oxidizing iron, followed by reducing the oxide film on the steel sheet surface in an atmosphere reducing iron. In particular, Fe in the steel sheet surface is oxidized at 400°C or higher using a direct fired burner with an air ratio of 0.93 to 1.10 and the steel sheet is then annealed in an N₂ + H₂ gas atmosphere reducing Fe oxides, whereby selective surface oxidation which deteriorates chemical conversion treatability is suppressed and an Fe oxidation layer is formed on the outermost surface. Patent Literature 6 does not particularly describe the heating temperature of the direct fired burner. When a large amount (about 0.6% or more) of Si is contained, the amount of oxidized Si, which is more likely to be oxidized than Fe, is large; hence, the oxidation of Fe is suppressed or is slight. As a result, the formation of a surface Fe reduction layer after reduction is insufficient or a lack of hiding is caused in a chemical conversion coating in some cases because SiO₂ is present on the steel sheet surface after reduction. WO 2014/0171010 discloses a method of heat treating a high strength steel plate having superior chemical conversion treatment properties and superior corrosion resistance after electrodeposition.

### Citation List

### Patent Literature

PTL 1: Japanese Unexamined Patent Application Publication No. 5-320952
PTL 2: Japanese Unexamined Patent Application Publication No. 2004-323969
PTL 3: Japanese Unexamined Patent Application Publication No. 6-10096
PTL 4: Japanese Unexamined Patent Application Publication No. 2003-113441
PTL 5: Japanese Unexamined Patent Application Publication No. 55-145122
PTL 6: Japanese Unexamined Patent Application Publication No. 2006-45615

### Summary of Invention

### Technical Problem

The present invention has been made in view of the above circumstances. It is an object of the present invention to provide a method for manufacturing the high-strength steel sheet as given in claim 1.

### Solution to Problem

Hitherto, an inner portion of a steel sheet containing oxidizable elements such as Si and Mn has been willingly oxidized for the purpose of improving the chemical conversion treatability thereof. However, this causes chemical conversion treatment unevenness or a lack of hiding on a surface because of the oxidation of the inner portion or deteriorates corrosion resistance after electrodeposition coating. Therefore, the inventors have investigated a method for solving this problem by a novel technique without being bound to conventional ideas. As a result, the inventors have found that the formation of internal oxides in a surface portion of a steel sheet is suppressed and excellent chemical conversion treatability and high corrosion resistance after electrodeposition coating are achieved in such a manner that the heating rate, atmosphere, and temperature in a heating step during continuous annealing are appropriately controlled. During continuous annealing, the steel sheet is annealed in such a manner that the steel sheet is heated at a heating rate of 7 °C/s or more in a temperature range corresponding to an annealing furnace inside temperature of 450°C to A°C (where 500 ≤ A ≤ 600), the maximum end-point temperature of the steel sheet in an annealing furnace is controlled to be 600°C to 700°C, the transit time of the steel sheet in a temperature range corresponding to a steel sheet temperature of 600°C to 700°C is controlled to be 30 seconds to 10 minutes, and the concentration of hydrogen in an atmosphere is controlled to be 20% by volume or more in the heating step. Subsequently, a chemical conversion treatment is performed. Since the heating rate in the temperature range corresponding to an annealing furnace inside temperature of 450°C to A°C (where 500 ≤ A ≤ 600) is 7 °C/s or more, the maximum end-point temperature of the steel sheet in the annealing furnace is 600°C to 700°C, and the concentration of hydrogen in the atmosphere in the temperature range corresponding to a steel sheet temperature of 600°C to 700°C is 20% by volume or more in the heating step, the potential of oxygen at the interface between the steel sheet and the atmosphere is reduced, internal oxidation hardly occurs, and the selective surface diffusion and oxidation (hereinafter referred to as surface oxidation) of Si, Mn, and the like are suppressed.

No internal oxide is formed and surface oxidation is minimized by controlling the heating rate of such a limited region only and the concentration of hydrogen in an atmosphere, whereby a high-strength steel sheet which is free from a lack of hiding and unevenness and which has excellent chemical conversion treatability and corrosion resistance after electrodeposition coating is obtained. The term "excellent chemical conversion treatability" refers to having an appearance free from a lack of hiding and unevenness after a chemical conversion treatment.

A high-strength steel sheet obtained by the above method includes a surface portion within 100 µm from a surface of the steel sheet. In the surface portion, the formation of the following oxide is suppressed: an oxide of one or more selected from among Fe, Si, Mn, Al, P, and further B, Nb, Ti, Cr, Mo, Cu, Ni, Sn, Sb, Ta, W, and V. The amount of the formed oxide per side is limited to less than 0.030 g/m² in total. This leads to excellence in chemical conversion treatability and a significant increase in corrosion resistance after electrodeposition coating.

The present invention is based on the above finding and is featured as described below.
(1) A method for manufacturing a high-strength steel sheet includes continuously annealing a steel sheet containing, by mass%, 0.03% to 0.35% C, 0.01% to 0.50% Si, 3.6% to 8.0% Mn, 0.01% to 1.0% Al, 0.10% or less P, and 0.010% or less S, the remainder being Fe and inevitable impurities. In a heating step, the steel sheet is heated at a heating rate of 7 °C/s or more in a temperature range corresponding to an annealing furnace inside temperature of 450°C to A°C (where 500 ≤ A ≤ 600), the maximum end-point temperature of the steel sheet in an annealing furnace is 600°C to 700°C, the transit time of the steel sheet in a temperature range corresponding to a steel sheet temperature of 600°C to 700°C is 30 seconds to 10 minutes, and the concentration of hydrogen in an atmosphere is 20% by volume or more.
(2) In the method for manufacturing the high-strength steel sheet specified in Item (1) above, the steel sheet further contains, by mass%, one or more selected from among 0.001% to 0.005% B, 0.005% to 0.05% Nb, 0.005% to 0.05% Ti, 0.001% to 1.0% Cr, 0.05% to 1.0% Mo, 0.05% to 1.0% Cu, 0.05% to 1.0% Ni, 0.001% to 0.20% Sn, 0.001% to 0.20% Sb, 0.001% to 0.10% Ta, 0.001% to 0.10% W, and 0.001% to 0.10% V as a component composition.
(3) The method for manufacturing the high-strength steel sheet specified in Item (1) or (2) above further includes performing electrolytic pickling in an aqueous solution containing sulfuric acid after the continuous annealing is performed.
(4) A high-strength steel sheet is manufactured by the method specified in any one of Items (1) to (3) above. The amount of an oxide of one or more selected from among Fe, Si, Mn, Al, P, B, Nb, Ti, Cr, Mo, Cu, Ni, Sn, Sb, Ta, W, and V per side is less than 0.030 g/m² in total, the oxide being formed in a surface portion of the steel sheet that is within 100 µm from a surface of the steel sheet.

A high-strength steel sheet according to the present invention has a tensile strength TS of 590 MPa or more. The term "high-strength steel sheet" as used herein includes both a cold-rolled steel sheet and a hot-rolled steel sheet. Advantageous Effects of Invention

According to the present invention, a high-strength steel sheet that has excellent chemical conversion treatability and corrosion resistance after electrodeposition coating is obtained even when the content of Si or Mn is high.

### Description of Embodiments

The present invention is described below in detail. In descriptions below, the unit of the content of each element in the steel composition is "mass percent" and is simply denoted by "%" unless otherwise specified.

First, annealing conditions which are the most important requirements for the present invention and which determine the surface structure of a steel sheet are described. In order to allow a high-strength steel sheet made from steel containing large amounts of Si and Mn to have satisfied corrosion resistance, the internal oxidation of a steel-sheet surface layer that may possibly be the origin of corrosion needs to be minimized. Chemical conversion treatability can be enhanced by promoting the internal oxidation of Si and Mn. However, this causes the deterioration of corrosion resistance as described above. Therefore, it is necessary that good chemical conversion treatability is maintained by a method other than promoting the internal oxidation of Si and Mn and corrosion resistance is enhanced by suppressing internal oxidation. As a result of intensive investigations, in the present invention, the potential of oxygen is reduced in an annealing step for the purpose of ensuring chemical conversion treatability and the activity of Si, Mn, and the like, which are oxidizable elements, in a base metal surface portion is reduced. This suppresses the external oxidation of these elements, resulting in improving chemical conversion treatability. Furthermore, the formation of internal oxides in a steel sheet surface portion is suppressed and therefore corrosion resistance after electrodeposition coating is improved.

Such an effect is obtained in such a manner that when annealing is performed in a continuous annealing line, the heating rate in a temperature range corresponding to an annealing furnace inside temperature of 450°C to A°C (where 500 ≤ A ≤ 600) is controlled to be 7 °C/s or more, the maximum end-point temperature of a steel sheet in an annealing furnace is controlled to be 600°C to 700°C, the transit time of the steel sheet in a temperature range corresponding to a steel sheet temperature of 600°C to 700°C is controlled to be 30 seconds to 10 minutes, and the concentration of hydrogen in an atmosphere is controlled to be 20% by volume or more in a heating step. Since heating is performed in such a manner that the heating rate in the temperature range corresponding to an annealing furnace inside temperature of 450°C to A°C (where 500 ≤ A ≤ 600) is controlled to be 7 °C/s or more, the formation of surface oxides is minimized. Since the concentration of hydrogen in the atmosphere is controlled to be 20% by volume or more in the temperature range corresponding to a steel sheet temperature of 600°C to 700°C, the potential of oxygen at the interface between the steel sheet and the atmosphere is reduced and the selective surface diffusion and surface oxidation of Si, Mn, and the like is suppressed without forming internal oxides. As a result, excellent chemical conversion treatability free from a lack of hiding and unevenness and high corrosion resistance after electrodeposition coating are achieved.

The reason why the temperature range in which the heating rate is controlled is 450°C or higher is as described below. In a temperature range lower than 450°C, surface oxidation and internal oxidation do not occur to such an extent that the occurrence of a lack of hiding and unevenness, the deterioration of corrosion resistance, and the like are problematic. Thus, the temperature range, in which an effect of the present invention is exhibited, is 450°C or higher.

The reason why the temperature range is A°C (where 500 ≤ A ≤ 600) or lower is as described below. In a temperature range lower than 500°C, the time for which the heating rate is controlled to be 7 °C/s or more is short and therefore an effect of the present invention is small. The effect of suppressing surface oxidation is insufficient. Therefore, A is 500 or more. The case of higher than 600°C is disadvantageous from the viewpoints of the deterioration of annealing furnace internals (rolls and the like) and an increase in cost, although there is no problem for an effect of the present invention. Thus, A is 600 or less.

The reason why the heating rate is 7 °C/s or more is as described below. The effect of suppressing surface oxidation is recognized when the heating rate is 7 °C/s or more. The upper limit of the heating rate is not particularly limited. When the heating rate is 500 °C/s or more, the above effect is saturated, which is disadvantageous in terms of cost. Therefore, the heating rate is preferably 500 °C/s or less. The heating rate can be adjusted to 7 °C/s or more in such a manner that, for example, an induction heater is placed in an annealing furnace in which the temperature of the steel sheet is 450°C to A°C.

The reason why the maximum end-point temperature of the steel sheet in the annealing furnace is 600°C to 700°C is as described below. When the maximum end-point temperature of the steel sheet is lower than 600°C, good material quality is not obtained. Therefore, a temperature range in which an effect of the present invention is exhibited is 600°C or higher. However, in a temperature range higher than 700°C, surface oxidation is significant and the deterioration of chemical conversion treatability is serious. Furthermore, in the temperature range higher than 700°C, the effect of balancing between strength and ductility is saturated from the viewpoint of material quality. From the above, the maximum end-point temperature of the steel sheet is 600°C to 700°C.

The reason why the transit time of the steel sheet in the temperature range corresponding to a steel sheet temperature of 600°C to 700°C is 30 seconds to 10 minutes is as described below. When the transit time of the steel sheet in the temperature range corresponding to a steel sheet temperature of 600°C to 700°C is less than 30 seconds, target material quality (TS, El) is not obtained. When the transit time of the steel sheet in the temperature range corresponding to a steel sheet temperature of 600°C to 700°C is more than 10 minutes, the effect of balancing between strength and ductility is saturated.

The reason why the concentration of hydrogen in the atmosphere in the temperature range corresponding to a steel sheet temperature of 600°C to 700°C is 20% by volume or more is as described below. The effect of suppressing surface oxidation begins to be recognized when the concentration of hydrogen is 20% by volume. The upper limit of the concentration of hydrogen is not particularly limited. When the concentration of hydrogen is more than 80% by volume, the above effect is saturated, which is disadvantageous in terms of cost. Therefore, the concentration of hydrogen is preferably 80% by volume or less.

The composition of the steel sheet of the high-strength steel sheet of the present invention are described below.

### C: 0.03% to 0.35%

C forms martensite and the like as a steel microstructure to enhance workability. Therefore, the content of C needs to be 0.03% or more. However, when the content of C is more than 0.35%, strength increases extremely and elongation decreases, resulting in the deterioration of workability. Thus, the content of C is 0.03% to 0.35%.

### Si: 0.01% to 0.50%

Although Si is an element that is effective in strengthening steel to obtain good material quality, Si is an oxidizable element and therefore is disadvantageous for chemical conversion treatability. Si is an element that should be avoided being added as much as possible. However, about 0.01% of Si is inevitably contained in steel. Reducing the content of Si to 0.01% or less leads to an increase in cost. From the above, the lower limit is 0.01%. On the other hand, when the content of Si is more than 0.50%, the effect of increasing the strength and elongation of steel is saturated and chemical conversion treatability is deteriorated. Thus, the content of Si is 0.01% to 0.50%.

### Mn: 3.6% to 8.0%

Mn is an element effective in increasing the strength of steel. In order to ensure mechanical properties and strength, 3.6% or more Mn needs to be contained. However, when more than 8.0% Mn is contained, it is difficult to ensure chemical conversion treatability and the balance between strength and ductility. Furthermore, there is a cost disadvantage. Thus, the content of Mn is 3.6% to 8.0%.

### Al: 0.01% to 1.0%

Al is added for the purpose of deoxidizing molten steel. When the content of Al is less than 0.01%, the purpose of deoxidizing molten steel is not achieved. The effect of deoxidizing molten steel is achieved when the content of Al is 0.01% or more. However, when the content of Al is more than 1.0%, an increase in cost is caused. Furthermore, the surface oxidation of Al is increased and it is difficult to improve chemical conversion treatability. Thus, the content of Al is 0.01% to 1.0%.

### P≤0.10%

P is one of inevitably contained elements. In order to adjust the content of P to less than 0.005%, an increase in cost may possibly be caused. Therefore, the content of P is preferably 0.005% or more. However, when more than 0.10% of P is contained, weldability is deteriorated. Furthermore, the deterioration of chemical conversion treatability is significant and it is difficult to enhance chemical conversion treatability even by the present invention. Thus, the content of P is 0.10% or less and the lower limit is preferably 0.005%.

### S≤0.010%

S is one of the inevitably contained elements. The lower limit is not particularly limited. When a large amount of S is contained, weldability and corrosion resistance are deteriorated. Therefore, the content of S is 0.010% or less.

In order to improve surface quality and to further improve the balance between strength and ductility, the following element may be added where appropriate: an element that is one or more selected from among 0.001% to 0.005% B, 0.005% to 0.05% Nb, 0.005% to 0.05% Ti, 0.001% to 1.0% Cr, 0.05% to 1.0% Mo, 0.05% to 1.0% Cu, 0.05% to 1.0% Ni, 0.001% to 0.20% Sn, 0.001% to 0.20% Sb, 0.001% to 0.10% Ta, 0.001% to 0.10% W, and 0.001% to 0.10% V.

In the case where these elements are added, the reason for limiting the appropriate amount of each added element is as described below.

### B: 0.001% to 0.005%

When the content of B is less than 0.001%, the effect of accelerating hardening is unlikely to be obtained. However, when the content of B is more than 0.005%, chemical conversion treatability is deteriorated. Thus, when B is contained, the content of B is 0.001% to 0.005%. Incidentally, in the case where the addition of B is judged to be unnecessary to improve mechanical properties, B need not be added.

### Nb: 0.005% to 0.05%

When the content of Nb is less than 0.005%, the effect of adjusting strength is unlikely to be obtained. However, when the content of Nb is more than 0.05%, an increase in cost is caused. Thus, when Nb is contained, the content of Nb is 0.005% to 0.05%.

### Ti: 0.005% to 0.05%

When the content of Ti is less than 0.005%, the effect of adjusting strength is unlikely to be obtained. However, when the content of Ti is more than 0.05%, the deterioration of chemical conversion treatability is caused. Thus, when Ti is contained, the content of Ti is 0.005% to 0.05%.

### Cr: 0.001% to 1.0%

When the content of Cr is less than 0.001%, a hardening effect is unlikely to be obtained. However, when the content of Cr is more than 1.0%, Cr is surface-oxidized and therefore weldability is deteriorated. Thus, when Cr is contained, the content of Cr is 0.001% to 1.0%.

### Mo: 0.05% to 1.0%

When the content of Mo is less than 0.05%, the effect of adjusting strength is unlikely to be obtained. However, when the content of Mo is more than 1.0%, an increase in cost is caused. Thus, when Mo is contained, the content of Mo is 0.05% to 1.0%.

### Cu: 0.05% to 1.0%

When the content of Cu is less than 0.05%, the effect of accelerating the formation of a retained γ-phase is unlikely to be obtained. However, when the content of Cu is more than 1.0%, an increase in cost is caused. Thus, when Cu is contained, the content of Cu is 0.05% to 1.0%.

### Ni: 0.05% to 1.0%

When the content of Ni is less than 0.05%, the effect of accelerating the formation of the retained γ-phase is unlikely to be obtained. However, when the content of Ni is more than 1.0%, an increase in cost is caused. Thus, when Ni is contained, the content of Ni is 0.05% to 1.0%.

### Sn: 0.001% to 0.20%, Sb: 0.001% to 0.20%

Sn and Sb may be contained from the viewpoint of suppressing the nitriding or oxidation of a surface of the steel sheet or the decarburization of a region of tens of micrometers in the steel sheet surface, the decarburization being due to oxidation. Suppressing the nitriding or oxidation thereof prevents the amount of martensite produced in the steel sheet surface from being reduced, thereby improving fatigue properties and surface quality. From the above viewpoint, when Sn and/or Sb is contained, the content of each of Sn and Sb is 0.001% or more. When the content of either of Sn and Sb is more than 0.20%, the deterioration of toughness is caused. Therefore, the content of each of Sn and Sb is preferably 0.20% or less.

### Ta: 0.001% to 0.10%

Ta forms a carbide and a carbonitride with C and N to contribute to increasing strength and also contributes to increasing yield ratio (YR). Ta has the property of refining the microstructure of a hot-rolled steel sheet. This property reduces the diameter of ferrite grains after cold rolling and annealing. Thus, the amount of C segregated along grain boundaries increases with the increase in area of the grain boundaries and a high bake hardening value (BH value) can be obtained. From this viewpoint, 0.001% or more Ta may be contained. However, containing more than 0.10% Ta causes an increase in material cost and may possibly interfere with the formation of martensite in the course of cooling after annealing. Furthermore, TaC precipitated in the hot-rolled steel sheet increases deformation resistance during cold rolling to make stable actual manufacture difficult in some cases. Thus, when Ta is contained, the content of Ta is 0.10% or less.

### W: 0.001% to 0.10%, V: 0.001% to 0.10%

W and V are elements which form a carbonitride and which have the property of increasing the strength of steel by a precipitation effect and may be added as required. In the case where W and/or V is added, this property is exhibited when the content of each of W and V is 0.001% or more. However, when more than 0.10% W and/or V is contained, strength is extremely increased and ductility is deteriorated. From the above, when W and/or V is contained, the content of each of W and V is 0.001% to 0.10%.

The remainder other than the above elements are Fe and inevitable impurities. If an element other than the above elements is contained, the present invention is not adversely affected. The upper limit of the element other than the above elements is 0.10%.

A method for manufacturing the high-strength steel sheet according to the present invention and the reason for limiting the method are described below.

Steel containing the above chemical components is hot-rolled, followed by cold rolling, whereby a steel sheet is obtained. The steel sheet is annealed in a continuous annealing line. Furthermore, the steel sheet is preferably electrolytically pickled in an aqueous solution containing sulfuric acid. The steel sheet is then subjected to a chemical conversion treatment. In the present invention, when the steel sheet is annealed, the heating rate in a temperature range corresponding to an annealing furnace inside temperature of 450°C to A°C (where 500 ≤ A ≤ 600) is 7 °C/s or more, the maximum end-point temperature of the steel sheet in an annealing furnace is 600°C to 700°C, the transit time of the steel sheet in a temperature range corresponding to a steel sheet temperature of 600°C to 700°C is 30 seconds to 10 minutes, and the concentration of hydrogen in an atmosphere is 20% by volume or more in a heating step. This is the most important requirement in the present invention. In the above, hot rolling is directly followed by annealing without performing cold rolling in some cases.

### Hot rolling

Hot rolling can be performed under conditions usually used.

### Pickling

Pickling is preferably performed after hot rolling. Mill scales formed on a surface are removed in a pickling step, followed by cold rolling. Pickling conditions are not particularly limited.

### Cold rolling

Cold rolling is preferably performed with a rolling reduction of 40% to 80%. When the rolling reduction is less than 40%, the recrystallization temperature is reduced and therefore mechanical properties are likely to be deteriorated. However, when the rolling reduction is more than 80%, not only rolling costs increase because of the high-strength steel sheet but also chemical conversion treatability is deteriorated because surface oxidation increases during annealing in some cases.

The cold-rolled or hot-rolled steel sheet is annealed and is then subjected to the chemical conversion treatment.

In the annealing furnace, the heating step is performed such that the steel sheet is heated to a predetermined temperature in an upstream heating zone and a soaking step is performed such that the steel sheet is held at a predetermined temperature for a predetermined time in a downstream soaking zone.

In the heating step, the heating rate in the temperature range corresponding to an annealing furnace inside temperature of 450°C to A°C (where 500 ≤ A ≤ 600) is 7 °C/s or more, the maximum end-point temperature of the steel sheet in an annealing furnace is 600°C to 700°C, the transit time of the steel sheet in the temperature range corresponding to a steel sheet temperature of 600°C to 700°C is 30 seconds to 10 minutes, and the concentration of hydrogen in the atmosphere is controlled to be 20% by volume or more as described above.

Gaseous components in the annealing furnace are nitrogen, hydrogen, and inevitable impurities. If no effect of the present invention is impaired, another gaseous component may be contained.

The concentration of hydrogen in a temperature range other than the temperature range corresponding to a steel sheet temperature of 600°C to 700°C, that is, a temperature range lower than 600°C or higher than 700°C, is not particularly limited. When the concentration of hydrogen therein is less than 1% by volume, no activation effect due to reduction is obtained and chemical conversion treatability is deteriorated in some cases. The upper limit is not particularly limited. When the upper limit is more than 50% by volume, an increase in cost is caused and an effect is saturated. Thus, the concentration of hydrogen therein is preferably 1% to 50% by volume and more preferably 5% to 30% by volume. The remainder are N₂ and inevitable impurity gases. If no effect of the present invention is impaired, a gaseous component such as H₂O, CO₂, or CO may be contained.

After cooling from the temperature range of 600°C to 700°C, quenching or tempering may be performed as required. Conditions are not particularly limited. Tempering is preferably performed at a temperature of 150°C to 400°C. This is because elongation tends to be deteriorated when the temperature is lower than 150°C and hardness tends to be reduced when the temperature is higher than 400°C.

In the present invention, even if electrolytic pickling is not performed, good chemical conversion treatability can be ensured. However, after continuous annealing is performed, electrolytic pickling is preferably performed in an aqueous solution containing sulfuric acid for the purpose of removing slight amounts of surface oxides inevitably formed during annealing to ensure better chemical conversion treatability.

A pickling solution used for electrolytic pickling is not particularly limited. Nitric acid and hydrofluoric acid are highly corrosive to equipment, requires caution in handling, and therefore are not preferable. Hydrochloric acid may possibly generate a chlorine gas from a cathode and therefore is not preferable. Thus, in consideration of corrosiveness and environments, sulfuric acid is preferably used. The concentration of sulfuric acid is preferably 5% to 20% by mass. When the concentration of sulfuric acid is less than 5% by mass, conductivity is low; hence, the voltage of an electrolytic bath rises during electrolysis to increase the load of a power supply in some cases. However, when the concentration of sulfuric acid is more than 20% by mass, the loss due to drag-out is large, which is problematic in terms of cost.

Conditions for electrolytic pickling are not particularly limited. In order to efficiently remove surface oxides, such as oxides of Si and Mn, formed after annealing and inevitably surface-oxidized, alternating electrolysis is preferably performed at a current density of 1 A/dm² or more. The reason for performing alternating electrolysis is as described below. When the steel sheet is being held as a cathode, a pickling effect is small. In contrast, when the steel sheet is being held as an anode, Fe dissolved during electrolysis is accumulated in the pickling solution and therefore the concentration of Fe in the pickling solution is increased; hence, a problem with dry stains or the like occurs if the pickling solution is attached to a surface of the steel sheet.

The temperature of an electrolytic solution is preferably 40°C to 70°C. The temperature of a bath is increased by heat generated by continuous electrolysis and therefore it is difficult to maintain the electrolytic solution at lower than 40°C in some cases. From the viewpoint of the durability of a lining of an electrolytic cell, it is not preferable that the temperature of the electrolytic solution exceeds 70°C. When the temperature of the electrolytic solution is lower than 40°C, the pickling effect is small. Therefore, the temperature of the electrolytic solution is preferably 40°C or higher.

The high-strength steel sheet according to the present invention is obtained as described above. The surface structure of the steel sheet is featured as described below.

In a surface portion of the steel sheet that is within 100 µm from a surface of the steel sheet, the amount of the following oxide per side is limited to less than 0.030 g/m² in total: an oxide of one or more selected from among Fe, Si, Mn, Al, P, B, Nb, Ti, Cr, Mo, Cu, Ni, Sn, Sb, Ta, W, and V.

In the steel sheet, which is made from steel containing large amounts of Si and Mn, it is required that the internal oxidation of a surface layer of a base steel sheet is minimized, chemical conversion treatment unevenness and a lack of hiding are suppressed, and corrosion and cracking during heavy machining are also suppressed. Therefore, in the present invention, the potential of oxygen is reduced in the annealing step for the purpose of ensuring good chemical conversion treatability, whereby the activity of Si, Mn, and the like, which are oxidizable elements, in a base metal surface portion is reduced. Furthermore, the external oxidation of these elements is suppressed and the formation of internal oxides in the base metal surface portion is also suppressed. As a result, not only good chemical conversion treatability is ensured but also workability and corrosion resistance after electrodeposition coating are enhanced. Such an effect is obtained in such a manner that in a surface portion of the steel sheet that is within 100 µm from a surface of the base steel sheet, the amount of the following oxide is limited to less than 0.030 g/m² in total: an oxide of at least one selected from among Fe, Si, Mn, Al, P, B, Nb, Ti, Cr, Mo, Cu, Ni, Sn, Sb, Ta, W, and V. When the sum (hereinafter referred to as the internal oxidation amount) of the amounts of formed oxides is 0.030 g/m² or more, not only corrosion resistance and workability are deteriorated but also chemical conversion treatment unevenness and a lack of hiding are caused. Even if the internal oxidation amount is limited to less than 0.0001 g/m², the effect of improving corrosion resistance and the effect of enhancing workability are saturated. Therefore, the lower limit of the internal oxidation amount is preferably 0.0001 g/m².

### EXAMPLES

The present invention is described below in detail with reference to examples.

Hot-rolled steel sheets with a steel composition shown in Table 1 were pickled, whereby mill scales were removed. Thereafter, the hot-rolled steel sheets were cold-rolled under conditions shown in Tables 2 and 3, whereby cold-rolled steel sheets with a thickness of 1.0 mm were obtained. Incidentally, after the mill scales were removed, some of the hot-rolled steel sheets (a thickness of 2.0 mm) were used without being cold-rolled.

**[Table 1]**

| (mass percent) | | | | | | | | | | | | | | | | | | |
|---|---|---|---|---|---|---|---|---|---|---|---|---|---|---|---|---|---|---|
| Steel symbol | C | Si | Mn | Al | P | S | Cr | Mo | B | Nb | Cu | Ni | Ti | Sn | Sb | Ta | W | V |
| A | 0.11 | 0.02 | 4.4 | 0.02 | 0.01 | 0.003 | - | - | - | - | - | - | - | - | - | - | - | - |
| B | 0.02 | 0.02 | 4.5 | 0.03 | 0.01 | 0.003 | - | - | - | - | - | - | - | - | - | - | - | - |
| C | 0.35 | 0.02 | 4.8 | 0.03 | 0.01 | 0.003 | - | - | - | - | - | - | - | - | - | - | - | - |
| D | 0.13 | 0.11 | 4.6 | 0.02 | 0.01 | 0.003 | - | - | - | - | - | - | - | - | - | - | - | - |
| E | 0.12 | 0.31 | 4.7 | 0.03 | 0.01 | 0.003 | - | - | - | - | - | - | - | - | - | - | - | - |
| F | 0.11 | 0.49 | 4.5 | 0.03 | 0.01 | 0.003 | - | - | - | - | - | - | - | - | - | - | - | - |
| G | 0.12 | 0.02 | 3.7 | 0.03 | 0.01 | 0,003 | - | - | - | - | - | - | - | - | - | - | - | - |
| H | 0.11 | 0.03 | 6.2 | 0.02 | 0.01 | 0.003 | - | - | - | - | - | - | - | - | - | - | - | - |
| I | 0.11 | 0.02 | 8.0 | 0.03 | 0.01 | 0.003 | - | - | - | - | - | - | - | - | - | - | - | - |
| J | 0.12 | 0.02 | 4.6 | 0.29 | 0.01 | 0.003 | - | - | - | - | - | - | - | - | - | - | - | - |
| K | 0.11 | 0.03 | 4.5 | 0.99 | 0.01 | 0.003 | - | - | - | - | - | - | - | - | - | - | - | - |
| L | 0.12 | 0.02 | 4.6 | 0.02 | 0.04 | 0.003 | - | - | - | - | - | - | - | - | - | - | - | - |
| M | 0.11 | 0.03 | 4.4 | 0.03 | 0.09 | 0.003 | - | - | - | - | - | - | - | - | - | - | - | - |
| N | 0.12 | 0.03 | 4.6 | 0.03 | 0.01 | 0.003 | - | - | - | - | - | - | - | - | - | - | - | - |
| O | 0.12 | 0.02 | 4.7 | 0.02 | 0.01 | 0.003 | 0.7 | - | - | - | - | - | - | - | - | - | - | - |
| P | 0.11 | 0.03 | 4.6 | 0.02 | 0.01 | 0.003 | - | 0.2 | - | - | - | - | - | - | - | - | - | - |
| Q | 0.12 | 0.02 | 4.6 | 0.03 | 0.01 | 0.003 | - | - | 0.002 | - | - | - | - | - | - | - | - | - |
| R | 0.11 | 0.03 | 4.5 | 0.04 | 0.01 | 0.003 | - | - | 0.002 | 0.02 | - | - | - | - | - | - | - | - |
| s | 0.12 | 0.02 | 4.6 | 0.02 | 0.01 | 0.003 | - | 0.2 | - | - | 0.2 | 0.1 | - | - | - | - | - | - |
| T | 0.12 | 0.03 | 4.7 | 0.03 | 0.01 | 0.003 | - | - | 0.002 | - | - | - | 0.01 | - | - | - | - | - |
| U | 0.11 | 0.02 | 4.7 | 0.04 | 0.01 | 0.003 | - | - | - | - | - | - | 0.04 | - | - | - | - | - |
| U1 | 0.12 | 0.02 | 4.5 | 0.02 | 0.01 | 0.003 | - | - | - | - | - | - | - | 0.04 | - | - | - | - |
| U2 | 0.11 | 0.03 | 4.6 | 0.03 | 0.01 | 0.003 | - | - | - | - | - | - | - | - | 0.03 | - | - | - |
| U3 | 0.12 | 0.03 | 4.5 | 0.03 | 0.01 | 0.003 | - | - | - | - | - | - | - | - | - | 0.02 | - | - |
| U4 | 0.11 | 0.03 | 4.6 | 0.02 | 0.01 | 0.003 | - | - | - | - | - | - | - | - | - | - | 0.02 | - |
| U5 | 0.12 | 0.03 | 4.7 | 0.02 | 0.0.1 | 0.003 | - | - | - | - | - | - | - | - | - | - | - | 0.02 |
| XA | 0.02 | 0.03 | 4.5 | 0.03 | 0.01 | 0.003 | - | - | - | - | - | - | - | - | - | - | - | - |
| XB | 0.36 | 0.02 | 4.6 | 0.03 | 0.01 | 0.003 | - | - | - | - | - | - | - | - | - | - | - | - |
| XC | 0.11 | 0.59 | 4.5 | 0.02 | 0.01 | 0.003 | - | - | - | - | - | - | - | - | - | - | - | - |
| XD | 0.12 | 0.02 | 3.5 | 0.03 | 0.01 | 0.003 | - | - | - | - | - | - | - | - | - | - | - | - |
| XE | 0.12 | 0.02 | 4.5 | 1.10 | 0.01 | 0.003 | - | - | - | - | - | - | - | - | - | - | - | - |
| XF | 0.11 | 0.03 | 4.6 | 0.03 | 0.11 | 0.003 | - | - | - | - | - | - | - | - | - | - | - | - |
| XG | 0.12 | 0.02 | 4.6 | 0.02 | 0.01 | 0.020 | - | - | - | - | - | - | - | - | - | - | - | - |
| XH | 0.11 | 0.02 | 8.1 | 0.02 | 0.01 | 0,003 | - | - | - | - | - | - | - | - | - | - | - | - |

| | | | | | | | | | | | | | | | | | | |
|---|---|---|---|---|---|---|---|---|---|---|---|---|---|---|---|---|---|---|
| Underlined items are outside the scope of the present invention. | | | | | | | | | | | | | | | | | | |

Next, each of the hot-rolled steel sheets and cold-rolled steel sheets obtained as described above was charged into a continuous annealing line. In the continuous annealing line, as shown in Tables 2 and 3, each steel sheet was processed and annealed by controlling the heating rate in a temperature range corresponding to a steel sheet temperature of 450°C to A°C (where 500 ≤ A ≤ 600) in an annealing furnace, the concentration of hydrogen in a temperature range corresponding to a steel sheet temperature of 600°C to 700°C in the annealing furnace, the transit time of the steel sheet, and the maximum end-point temperature of the steel sheet, followed by water quenching and then tempering at 300°C for 140 seconds. Subsequently, the steel sheet was pickled in such a manner that the steel sheet was immersed in a 40°C aqueous solution containing 5% by mass sulfuric acid. Some of the steel sheets were electrolytically pickled under current density conditions shown in Tables 2 and 3 by alternating electrolysis in such a manner that a specimen was held as an anode and a cathode in that order for 3 seconds, whereby specimens were obtained. The concentration of hydrogen in the annealing furnace other than a region where the concentration of hydrogen was controlled as described above was basically 10% by volume. Gaseous components in an atmosphere were a nitrogen gas, a hydrogen gas, and inevitable impurity gases. The dew point of the atmosphere was controlled by absorbing or removing moisture in the atmosphere. The dew point of the atmosphere was -35°C.

The specimens obtained as described above were measured for TS and El. Furthermore, the specimens were investigated for chemical conversion treatability and corrosion resistance after electrodeposition coating. The amount (internal oxidation amount) of oxides present in a surface portion of each steel sheet, the surface portion being located directly under a surface layer of the steel sheet and being within 100 µm from the surface layer, was measured. Measurement methods and evaluation standards are as described below.

### Chemical conversion treatability

A chemical conversion solution used was a chemical conversion solution (PALBOND® L3080) produced by Nihon Parkerizing Co., Ltd. Each specimen was subjected to a chemical conversion treatment by a method below. The specimen was degreased with a degreasing solution, FINECLEANER®, produced by Nihon Parkerizing Co., Ltd.; was washed with water; was surface-modified with a surface modifier, PREPALENE® Z, produced by Nihon Parkerizing Co., Ltd. for 30 seconds; was immersed in the chemical conversion solution (PALBOND® L3080) at 43°C for 120 seconds; was washed with water; and was then dried with hot air. Randomly selected five fields of view of the specimen subjected to the chemical conversion treatment were observed with a scanning electron microscope (SEM) at 500x magnification. The area fraction of a lack of hiding in a chemical conversion coating was measured by image processing. The specimen was evaluated depending on the area fraction of a lack of hiding as described below. "A" is an acceptable level.
A: 10% or less
B: more than 10%

### Corrosion resistance after electrodeposition coating

A test piece with a size of 70 mm × 150 mm was cut out of each specimen, obtained by the above method, subjected to the chemical conversion treatment, followed by cationic electrodeposition coating (baking conditions: 170°C for 20 minutes, a thickness of 25 µm) using PN-150G® manufactured by Nippon Paint Co., Ltd. Thereafter, end portions and a surface not evaluated were sealed with an Al tape and cross cuts (a cross angle of 60°) were made with a cutter knife so as to reach a base metal, whereby a specimen was prepared. Next, the specimen was immersed in a 5% aqueous solution of NaCl (55°C) for 240 hours, was taken out, was washed with water, and was then dried, followed by peeling the tape from a cross cut portion. The separation width was measured and was evaluated as described below. "A" is an acceptable level.
A: a separation width of less than 2.5 mm per side
B: a separation width of 2.5 mm or more per side Workability

A JIS #5 tensile test piece was taken from each sample in a 90° direction with respect to a rolling direction and was measured for workability in such a manner that tensile testing was performed at a constant cross head speed of 10 mm/min in accordance with JIS Z 2241 and the tensile strength (TS/MPa) and elongation (El/%) were determined. A test piece satisfying the inequality TS × El ≥ 18,000 was rated good. A test piece satisfying the inequality TS × El < 18,000 was rated poor.

### Internal oxidation amount in region within 100 µm from surface layer of steel sheet

The internal oxidation amount was measured by "impulse furnace fusion-infrared absorption spectrometry". Incidentally, the amount of oxygen contained in steel (that is, an unannealed high-strength steel sheet) needs to be subtracted. Therefore, in the present invention, surface portions of both sides of each continuously annealed high-strength steel sheet were polished by 100 µm or more, the concentration of oxygen in steel was measured, and the measurement was defined as the oxygen amount OH in steel. Furthermore, the concentration of oxygen in steel was measured over the continuously annealed high-strength steel sheet in a thickness direction and the measurement was defined as the oxygen amount OI after internal oxidation. The difference between OI and OH (= OI - OH) was calculated using the oxygen amount OI of the high-strength steel sheet, obtained as described above, after internal oxidation and the oxygen amount OH in steel. Furthermore, a value (g/m²) converted into an amount per unit area (that is, 1 m²) per side was defined as the internal oxidation amount.

Results obtained as described above are shown in Tables 2 and 3 together with manufacturing conditions.

As is clear from Tables 2 and 3, high-strength steel sheets manufactured by a method according to the present invention has excellent chemical conversion treatability, corrosion resistance after electrodeposition coating, and workability, although the high-strength steel sheets contain large amounts of oxidizable elements such as Si and Mn. However, in comparative examples, one or more of chemical conversion treatability, corrosion resistance after electrodeposition coating, and workability are inferior.

### Industrial Applicability

A high-strength steel sheet according to the present invention has excellent chemical conversion treatability, corrosion resistance, and workability and can be used as a surface-treated steel sheet for lightening and strengthening automobile bodies. The high-strength steel sheet can be used in various fields, such as home appliances and building materials, other than automobiles in the form of a surface-treated steel sheet manufactured by imparting rust resistance to a base steel sheet.

## Claims

1. A method for manufacturing a high-strength steel sheet, comprising continuously annealing a steel sheet containing, by mass%, 0.03% to 0.35% C, 0.01% to 0.50% Si, 3.6% to 8.0% Mn, 0.01% to 1.0% Al, 0.10% or less P, and 0.010% or less S, and optionally one or more selected from among 0.001% to 0.005% B, 0.005% to 0.05% Nb, 0.005% to 0.05% Ti, 0.001% to 1.0% Cr, 0.05% to 1.0% Mo, 0.05% to 1.0% Cu, 0.05% to 1.0% Ni, 0.001% to 0.20% Sn, 0.001% to 0.20% Sb, 0.001% to 0.10% Ta, 0.001% to 0.10% W, and 0.001% to 0.10% V, the remainder being Fe and inevitable impurities, wherein in a heating step, the steel sheet is heated at a heating rate of 7°C/s or more in a temperature range corresponding to an annealing furnace inside temperature of 450°C to A°C (where 500 ≤ A ≤ 600), the maximum end-point temperature of the steel sheet in an annealing furnace is 600°C to 700°C, the transit time of the steel sheet in a temperature range corresponding to a steel sheet temperature of 600°C to 700°C is 30 seconds to 10 minutes, and the concentration of hydrogen in an atmosphere is 20% by volume or more.

2. The method for manufacturing the high-strength steel sheet according to Claim 1, further comprising performing electrolytic pickling in an aqueous solution containing sulfuric acid after the continuous annealing is performed.

## Patentansprüche

1. Verfahren für die Herstellung einer Platte aus hochfestem Stahl, umfassend das kontinuierliche Glühen einer Stahlplatte enthaltend, in Masse-%, 0,03 % bis 0,35 % C, 0,01 % bis 0,50 % Si, 3,6 % bis 8,0 % Mn, 0,01 % bis 1,0 % Al, 0,10 % Al, 0,10 % oder weniger P und 0,010 % oder weniger S und wahlweise eines oder mehrere ausgewählt unter 0,001 % bis 0,005 % B, 0,005 % bis 0,05 % Nb, 0,005 % bis 0,05 % Ti, 0,001 % bis 1,0 % Cr, 0,05 % bis 1,0 % Mo, 0,05 % bis 1,0 % Cu, 0,05 % bis 1,0 % Ni, 0,001 % bis 0,20 % Sn, 0,001 % bis 0,20 % Sb, 0,001 % bis 0,10 % Ta, 0,001 % bis 0,10 % W und 0,001 % bis 0,10 % V, wobei der Rest Fe und unvermeidliche Verunreinigungen ist, wobei in einem Erhitzungsschritt die Stahlplatte mit einer Erhitzungsrate von 7 °C/s oder mehr in einem Temperaturbereich, der der Innentemperatur eines Härteofens von 450 °C bis A °C (wobei 500 ≤ A ≤ 600), entspricht, erhitzt wird, wobei die maximale Endpunkttemperatur der Stahlplatte in einem Härteofen 600 °C bis 700 °C beträgt, die Übergangszeit der Stahlplatte in einem Temperaturbereich, der einer Stahlplattentemperatur von 600 °C bis 700 °C entspricht, 30 Sekunden bis 10 Minuten beträgt und die Wasserstoffkonzentration in einer Atmosphäre 20 Volumen-% oder mehr beträgt.

2. Verfahren für die Herstellung der Platte aus hochfestem Stahl nach Anspruch 1, ferner das Ausführen von elektrolytischem Beizen in einer wässrigen Lösung, die Schwefelsäure enthält, nachdem das kontinuierliche Glühen ausgeführt worden ist, umfassend.

## Revendications

1. Procédé de fabrication d'une tôle d'acier à haute résistance, comprenant un recuit continu d'une tôle d'acier contenant, en % en masse, 0,03 % à 0,35 % de C, 0,01 % à 0,50 % de Si, 3,6 % à 8,0 % de Mn, 0,01 % à 1,0 % d'Al, 0,10 % ou moins de P, et 0,010 % ou moins de S, et de manière facultative un ou plusieurs composés choisis parmi 0,001 % à 0,005 % de B, 0,005 % à 0,05 % de Nb, 0,005 % à 0,05 % de Ti, 0,001 % à 1,0 % de Cr, 0,05 % à 1,0 % de Mo, 0,05 % à 1,0 % de Cu, 0,05 % à 1,0 % de Ni, 0,001 % à 0,20 % de Sn, 0,001 % à 0,20 % de Sb, 0,001 % à 0,10 % de Ta, 0,001 % à 0,10 % de W, et 0,001 % à 0,10 % de V, le reste étant Fe et des impuretés inévitables, dans lequel, lors d'une étape de chauffage, la tôle d'acier est chauffée à une vitesse de chauffage de 7 °C/s ou plus dans une plage de température correspondant à une température intérieure de four de recuit de 450 °C à A °C (où 500 ≤ A ≤ 600), la température finale maximale de la tôle d'acier dans un four de recuit est de 600 °C à 700 °C, le temps de séjour de la tôle d'acier dans une plage de température correspondant à une température de tôle d'acier de 600 °C à 700 °C est de 30 secondes à 10 minutes, et la concentration en hydrogène dans une atmosphère est de 20 % en volume ou plus.

2. Procédé de fabrication de la tôle d'acier à haute résistance selon la revendication 1, comprenant en outre d'effectuer un décapage électrolytique dans une solution aqueuse contenant de l'acide sulfurique après le recuit continu.
